

March 15, 1932.

G. A. RICHTER

1,849,334

## PROCESS FOR THE PRODUCTION OF CHEMICAL WOOD PULP

Filed May 1, 1926



Inventor  
George A. Richter  
by  
Wright Brown, Shirley & May  
Atlys

## UNITED STATES PATENT OFFICE

GEORGE A. RICHTER, OF BERLIN, NEW HAMPSHIRE, ASSIGNOR TO BROWN COMPANY, OF  
BERLIN, NEW HAMPSHIRE, A CORPORATION OF MAINE

## PROCESS FOR THE PRODUCTION OF CHEMICAL WOOD PULP

Application filed May 1, 1928. Serial No. 105,995.

This invention relates to the production of chemical wood pulp as effected by well-known chemical pulping processes. Inasmuch as the present invention is especially 5 advantageous in the sulphite process, it will be described as applied thereto.

In producing sulphite pulp for use in the manufacture of bond, ledger and writing papers, a prime desideratum is fiber of good 10 strength and other physical characteristics. This is notably the case when the fiber is to serve as a raw material for the production of a high alpha cellulose fiber which is intended for use as a "new rag" substitute in the man- 15 ufacture of paper.

In order to appreciate the results obtained by the practice of the present invention, it is desirable preliminarily to consider certain factors that affect the production of sulphite 20 pulp. Initially, the wood, e. g., spruce, is cut into small, thin chips of more or less definite size. The chips, together with an acid sul- 25 phite liquor of the desired composition (usu- ally a calcium bi-sulphite liquor), are charged into a digester. The liquor usually contains about 5% free  $\text{SO}_2$  and 1% combined  $\text{SO}_2$ . The charge is slowly and gradually heated, as it is necessary to avoid a too rapid increase in temperature. Thus, 30 the operator may reach the maximum temperature of digestion of, say, from 205° to 310° F., in about eight to twelve hours after digestion was commenced. The maximum pressure of digestion is usually controlled by 35 the periodical opening of a relief valve at the top of the digester, which allows the escape of free sulphur dioxide and steam. Unless a time-temperature curve determined from experience is carefully adhered to and 40 the temperature thereon indicated at any definite time not exceeded, a fiber of inferior quality is produced. Injury to the fiber ensues because the combined  $\text{SO}_2$  is not given sufficient time to penetrate into the chips, 45 whereas the free  $\text{SO}_2$  diffuses readily thereinto and is present alone. In other words, the combined  $\text{SO}_2$  in the form of  $\text{SO}_3^-$  ions is not present in the chips in sufficient amount 50 to repress the ionization of the  $\text{H}_2\text{SO}_3$  into  $\text{H}^+$

ions, which hydrolyze and dissolve a portion of the fiber with an attendant low yield of short fiber pulp having low strength and tear resistance. By adhering to the predetermined time-temperature curve during the 55 digestion, sufficient time is allowed for penetration of combined  $\text{SO}_2$  into the chips.

Another factor which affects the rate of penetration of combined  $\text{SO}_2$  content into the chips is the concentration of combined 60  $\text{SO}_2$  in the digesting liquor. Thus, by increasing the combined  $\text{SO}_2$  content of the digesting liquor, the rate of penetration of combined  $\text{SO}_2$  into the chips may be increased. In the usual calcium base cooking liquor, however, the concentration of combined  $\text{SO}_2$  should not be raised above the concentration of a saturated solution thereof, which amounts to about 1%, for the reason that if saturation concentration is exceeded, 70 a heavy precipitate of calcium monosulphite is present during digestion, and the resulting pulp becomes contaminated with the precipitate.

The object of the present invention is to 75 avoid the long time heretofore necessary to reach maximum digesting temperature, without, however, sacrificing the quality of fiber. I have found that this object may be attained if the chips are suitably pre-treated or 80 chemically conditioned prior to digestion. I have further found that by suitable pre-treatment much larger wood chips may be digested without extending the time of digestion hertofore found necessary in producing 85 pulp with chips of usual size.

Briefly stated, in accordance with the process of this invention, the chips are immersed or soaked prior to digestion in a concentrated solution until they contain a total quantity of 90 combined  $\text{SO}_2$ , or of a base chemical capable of reacting with free  $\text{SO}_2$  to produce combined  $\text{SO}_2$ , even greater than that present in the standard acid cooking liquors employed 95 in the sulphite cooking process, which standard liquors have a combined  $\text{SO}_2$  content of about 1% as hereinbefore described. The chips may then be charged in a digester together with the desired amount of only water and free  $\text{SO}_2$ , and cooked under pressure

and at an elevated temperature until fiber liberation has been effected.

The pre-treating solution is not necessarily related to the cooking liquor subsequently employed in the digester, except that such solution is far more concentrated in the sense that it contains per unit volume of chips treated therewith an amount of combined SO<sub>2</sub> or of base chemical greater than that present in the usual or standard acid sulphite cooking liquor. Preferably, the pre-treating solution is highly concentrated or even saturated with the particular pre-treating chemical chosen, whereby the chips may acquire in a short period of time within their pores and interstices substantially all of the chemical other than SO<sub>2</sub> necessary for subsequent cooking to complete fiber liberation in the digester. The pre-treating solution may, for example, contain 20% sodium sulphite (10% combined SO<sub>2</sub>), and be prepared by combining a solution of sodium carbonate, caustic soda, or the like, with sulphur burner gas or with sulphur dioxide recovered from the blowpit or relief gases. Inasmuch as a sodium sulphite solution is neutral or faintly alkaline, ordinary apparatus is suitable for carrying out a pre-treatment with the solution. The pre-treatment should, however, be carried out in acid-proof apparatus when a sulphurous acid solution of sodium sulphite, say, a sodium bisulphite solution containing 10% free and 10% combined SO<sub>2</sub> is used. This latter procedure, using a liquor containing free SO<sub>2</sub>, tends to speed up the rate of penetration of combined SO<sub>2</sub> into the chips, but the use of a neutral or alkaline solution is generally more economical and expedient.

The chips are immersed or soaked in the pre-treating solution of sodium sulphite until they contain in their pores and interstices the desired combined SO<sub>2</sub> content, preferably substantially equal to that required for subsequent digestion and fiber liberation. The pre-treatment may be, and preferably is, carried on as a continuous operation at room or at elevated temperature (say, 200° to 212° F.), and under atmospheric pressure. If desired, however, a pressure somewhat above atmospheric may be applied to shorten the time of pre-treatment. Pre-treatment under pressure, however, is generally less desirable, inasmuch as it calls for the use of stronger apparatus and ordinarily can be practiced only as a batch basis.

After pre-treatment, the chips are removed from the solution and drained, whereupon they may then be stored in a chip loft or directly charged into a digester. The liquor drained from the chips may be recovered and re-employed in pretreating fresh chips after replenishment with an amount of water and chemical equivalent to that absorbed by the chips. The drained liquor will vary from a pale yellow color to a dark brown or

amber color, owing to partial solution or extraction of resinous and gummy materials from the chips. The coloring material, however, does not interfere with the pre-treatment of fresh chips.

The factors entering into the pre-treatment may, of course, be varied according to the type of pulp which it is desired to produce. Thus, in producing a "4-4" pulp such as described in my application, Serial No. 749,564, filed November 12, 1924, a quantity of chemical much higher than usual should be introduced into the chips by the pre-treatment. This may be accomplished by maintaining a suitable concentration of dissolved chemical in the pre-treating solution and by properly controlling the time and temperature of pre-treatment.

When the chips have acquired during pre-treatment the amount of base chemical or combined SO<sub>2</sub> necessary for digestion, only a sulphurous acid solution containing the desired SO<sub>2</sub> content is necessary for digestion. When the chips have acquired both the free and combined SO<sub>2</sub> content necessary for digestion, only water need be added to the digester to produce a cooking solution of the desired strength. The concentration of

+

ions within the chips during digestion, in either case, is sufficient to hydrolyze or dissolve the encrusting material or ligno-celluloses, but the chips also contain at the very start the necessary amount of combined SO<sub>2</sub> to avoid injury to the pulp, so that maximum temperature of digestion may be reached as rapidly as plant conditions will allow.

After fiber liberation has been effected, the digester contents may be blown, and the pulp separated from the spent liquor. The spent liquor may then be concentrated, its inorganic content smelted, and the smelted compounds recovered in aqueous solution. If desired, instead of re-using the solution drained from the chips after pre-treatment, it may be commingled with the spent liquor and the mixture subjected to recovery operations.

It should be noted that sodium is selected as the pre-treating base because its compounds are highly soluble in water and can give a high rate of penetration into the chips. The rate of penetration possible with calcium bisulphite, on the other hand, is materially lower, because of its low solubility and the consequent low concentration obtainable in a saturated solution thereof. The sodium compounds may be replaced in part or in whole by compounds of other bases which are highly soluble in water, such, for example, as magnesium sulphite, magnesium bisulphite, magnesium sulphate, or the like.

When the chips are pre-treated with a base chemical, such as caustic soda or sodium carbonate, then, during subsequent acid diges-

tion, the free  $\text{SO}_2$  introduced into the digester readily diffuses into the chips and immediately combines with the base chemical to produce combined  $\text{SO}_2$  in situ in the chips. 5 When the chips are pre-treated with a concentrated solution of sodium sulphate (salt cake), subsequent digestion will take place in a sulphurous acid solution of sodium sulphate, as described in my Patent No. 1,427, 10 125, dated August 29, 1922, should the added liquor consist of a sulphurous acid solution. When sodium sulphite or other suitable base chemical is employed in the pre-treatment of the chips, a sulphurous acid solution of 15 calcium sulphite may subsequently be introduced with the pre-treated chips into the digester, in which case digestion takes place in a composite base liquor, as described in my application for patent, Serial No. 94,621, filed 20 March 13, 1926.

It should be observed that the chips, if pre-treated at an elevated temperature, may be charged while in heated condition into the digester, thus conserving their heat content. 25 Where storage of the chips is necessary, however, even if partial evaporation of water from the chips ensues, the chemical remains entrapped therein.

One of the great advantages in practicing 30 a process such as hereinbefore described is that a material saving in time of digestion may be effected. The digesting period heretofore found necessary to produce a high quality sulphite fiber may be shortened to 35 from two to four hours without sacrificing quality of fiber. Moreover, pre-treated chips of larger than usual size may be successfully digested, but, inasmuch as more time is required to heat such chips, the time of digestion 40 may not be reduced below that heretofore found to be necessary. A pulp of exceedingly high strength and tear may be produced, however, by such latter practice, because the presence of short chips having short fibers and shives is largely eliminated. An increase of 45 about 25% in strength and tear may be realized in actual practice.

On the accompanying drawing, I have illustrated a schematic or conventional layout of apparatus which may be employed for 50 continuously carrying out the process of the present invention.

Now, describing the process as carried out 55 when sodium sulphite is employed as the specific pre-treating chemical, at 1 is shown a tower in which the pre-treating solution of sodium sulphite may be prepared. The tower may be filled with inert interstitial material, e. g., spiral brick, through which a 60 solution of caustic soda or soda ash may slowly percolate in counter-current contact with sulphur dioxide passed upwardly therethrough. The alkaline solution may be introduced at the top of the tower through a 65 valved pipe 2, and the sulphur dioxide may

be passed into the lower portion of the tower through a valved pipe 3,—the relative rates of flow and concentrations of these materials being regulated to produce a neutral sulphite liquor of high concentration at the bottom of 70 the tower. The sulphur dioxide employed may be sulphur burner gas or that recovered from the blowpit or relief gases, the inert gas carried along therewith into the tower being wasted through a vent 4. The sodium 75 sulphite solution may collect as a pool at the bottom of the tower and may be withdrawn by a pump 5 and delivered through a valved pipe 6 into a storage tank 7 in amount and concentration sufficient to replace the sodium sulphite and water absorbed 80 by the chips after pre-treatment and draining.

The pre-treatment of the chips may be carried out continuously in a rotary drum indicated conventionally as a whole at 8. The 85 chips may be continuously carried in predetermined, measured amount from the chipping machine on a belt conveyor 9, and charged into a hopper 10 feeding into the 90 intake end of the drum. The solution of sodium sulphite maintained at the proper concentration in the storage tank 7 may be withdrawn by a pump 11a and delivered at 95 predetermined rate into the intake end of the drum, together with the chips. The 100 chips may be continuously passed through the solution of sodium sulphite maintained in the drum at a rate such that when they issue from the drum they contain the combined  $\text{SO}_2$  content necessary for subsequent digestion.

The pre-treated chips may be continuously discharged through an inclined discharge 105 nose 11 at the outlet end of the drum on an inclined foraminous platform 12, the solution associated with the pre-treated chips 110 draining through the platform into a funnel 13 discharging into a pipe 14 leading to the storage tank 7. The solution draining from the chips is thus re-employed in the pre-treatment of other chips after sufficient fresh solution, which replaces the chemical and water absorbed by the chips after drainage, has 115 been admixed therewith. It may be desired, as previously stated, to carry out the pre-treatment of the chips at an elevated temperature, especially when a neutral or alkaline solution is employed in the pre-treatment. In this event, the treating liquor may be 120 heated to the desired temperature while in storage tank 7, prior to delivery into the treating drum, as by steam delivered into the tank from a steam line 7a. The drained chips may be conveyed to the chip loft or 125 discharged directly into the digester. As shown, the chips gravitate from the platform 12 onto a belt conveyor 15 which discharges into a continuous bucket elevator 16, which elevates the chips and then dumps them into 130

a loft 17, from which the chips may be removed, as required, for charging into a digester 18.

I claim:

- 5 1. A process which comprises treating chipped wood until it is completely permeated with a solution of at least about 10% concentration of a highly soluble compound capable of being converted by sulphurous acid into bisulphite, treating the permeated wood with only water and sulphur dioxide to produce a bisulphite cooking liquor of at least 1% strength in base, and cooking at elevated temperature and under pressure in the liquor to effect a liberation of fiber from the wood.
- 10 2. A process which comprises treating chipped wood until it is completely permeated with a solution of at least about 10% concentration of a sodium compound capable of being converted by sulphurous acid into bisulphite, treating the permeated wood with only water and sulphur dioxide to produce a bisulphite cooking liquor of at least 1% strength in sodium base, and cooking at elevated temperature and under pressure in the liquor to effect a liberation of fiber from the wood.
- 15 3. A process which comprises treating chipped wood until it is completely permeated with a solution of sodium sulphite of at least about 10% strength, treating the permeated wood with only water and sulphur dioxide to produce a bisulphite cooking liquor having a combined  $SO_2$  content of at least about 1%, and cooking at elevated temperature and under pressure in the liquor to effect a liberation of fiber from the wood.

In testimony whereof I have affixed my signature.

40 GEORGE A. RICHTER.

45

50

55

60

65